

# UNITED STATES PATENT OFFICE.

ARTUR KRUPP, OF BERNDORF, AUSTRIA-HUNGARY.

## PROCESS OF SMELTING NICKEL AND COBALT ORES.

### SPECIFICATION forming part of Letters Patent No. 308,175, dated November 18, 1884.

Application filed January 31, 1884. (No specimens.) Patented in France January 12, 1884, No. 159,690; in Germany January 15, 1884, No. 28,089; in Belgium January 15, 1884, No. 63,842; in England January 15, 1884, No. 1,464; in Italy January 15, 1884, XVII, 16,333, and XXXII, 311, and in Sweden March 26, 1884.

*To all whom it may concern:*

Be it known that I, ARTUR KRUPP, of  
Essen, in the German Empire, Prussia, sub-  
ject of the Emperor of the German Empire,  
5 residing at Berndorf, in the Province of Nether  
Austria, in the Empire of Austria-Hungary,  
have invented certain new and useful Improve-  
ments in Process of Smelting Nickel and Co-  
balt Ores; and I do hereby declare the follow-  
10 ing to be a full, clear, and exact description  
of the invention, such as will enable others  
skilled in the art to which it appertains to  
make and use the same.

This invention relates to a novel process of  
15 treating nickel or cobalt in order to obtain  
a homogeneous malleable or ductile metal.  
The affinity of nickel and cobalt for or their  
tendency to absorb or assimilate carbon as  
well as oxygen or both within certain lim-  
20 its has heretofore been the cause of failure to  
obtain a homogeneous and malleable cast  
metal. When smelted in a graphite crucible,  
these metals will combine with more or less  
carbon and oxygen, and the cast metal on cool-  
25 ing will give up the greater portion of oxygen,  
while the carbon is retained. The brittleness of  
the metal as well as the degree of ductility or  
malleability thereof will depend upon the  
amount of carbon combined therewith. It is,  
30 however, very easy to eliminate the oxygen  
during the process of smelting by keeping the  
metal in fusion for some time, and especially  
by smelting under a layer or strata of char-  
coal. This will, however, tend to increase its  
35 brittleness. The longer the metal is kept in  
fusion under these conditions the greater will  
be its brittleness, the grayer its color, and the  
nearer it will approach in texture to that of  
cast-iron, as the amount of carbon assimilated  
40 increases with the time the metal is kept in  
fusion, and such metal will be unfit for use for  
most purposes. In general I may say that  
when nickel or cobalt is smelted in presence  
of carbon, as in graphite crucibles, and I am  
45 not aware that crucibles free from carbon have  
ever been produced for this purpose, the ab-  
sorption or assimilation of the carbon is so  
rapid that unless prevented or counteracted  
the metal is always brittle or cast-iron like

and unfit for general use, owing to the carbon 50  
in the metal.

My improved process hereinafter described  
is based upon the properties of nickel and  
cobalt to assimilate or absorb both oxygen and  
carbon, and I obtain a thoroughly homogene- 55  
ous malleable or ductile product adapted for  
general use in the arts and manufactures. In  
order to obtain such homogeneous malleable  
nickel or cobalt, it is necessary to employ means  
to prevent the absorption or assimilation of 60  
carbon. This I have found can be attained by  
effecting the smelting of the metals in the ordi-  
nary graphite crucibles in presence of an  
oxidizing agent in such manner that the latter  
will gradually give up its oxygen as the smelt- 65  
ing progresses. Various oxidizing agents may  
be employed. I have, however, obtained the  
best results with a manganate or permanga-  
nate salt, preferably permanganate of potash  
and permanganate of soda, and in practice 70  
after the smelting is completed I preferably  
employ a deoxidizing agent to counteract the  
effect of the oxygen on these metals.

In carrying out my invention I take the  
oxide of nickel or cobalt in as pure a state as 75  
possible, and either in the form of cubes or  
small pieces of other form, and reduce them  
at a moderate heat to avoid fusing, and also to  
avoid their assimilating or absorbing carbon.  
The somewhat porous material thus obtained 80  
is then impregnated or saturated with a solu-  
tion of permanganate, either of soda or of  
potash, containing about four per cent. of the  
salt. The saturated material is then dried  
and smelted (preferably in a crucible) in a 85  
blast-furnace at a high temperature, the per-  
manganate counteracting the deleterious effect  
of the carbon of the gases evolved, and is it-  
self partially reduced, while the metal becomes  
homogeneous and malleable. 90

It is evident that by treating the reduced  
oxides as described, the oxidizing agent is in-  
timately incorporated therein, and in a finely-  
subdivided condition, and will, as the smelt-  
ing proceeds, be gradually given up, acting 95  
constantly to counteract the carbon and pre-  
vent it being absorbed by the metal. The ef-  
fect of the oxidizing agent is due more to the ab-

sorption of the liberated oxygen by the carbon than to the fact that the deleterious action on the metal of the small quantity of carbon absorbed thereby, notwithstanding any precaution that may be taken to prevent this is counteracted.

The metal may be completely deoxidized by any suitable agent—as, for instance, by the addition of black flux and charcoal. The former can be obtained by carefully heating tar-tar (bitartrate of potassia) in a closed vessel, or by the addition of small quantities of aluminium, calcium, or calcium-zinc, which latter can be readily obtained by the Caron process, 15 or by a mixture of any two or more of the latter metals.

In deoxidizing by means of black flux and charcoal these are introduced in small quantities either as soon as the metal has become 20 fluid or immediately after, and the combined action of the carbon and the potassium vapors evolved by the black flux will in a short time remove any oxygen combined with the metal.

In deoxidizing by means of the metals above 25 referred to I proceed as follows: I place on the fluid nickel or cobalt sufficient charcoal until it appears covered thereby, then through the charcoal I add the aluminium, or calcium, or calcium-zinc, or any two or more of these in 30 the proportion of about four parts of the latter to every one hundred parts of the molten metal. In this manner I obtain nickel or cobalt in a perfectly homogeneous and ductile or malleable form.

35 I am aware that permanganate of soda has

heretofore been used in the treatment of metals, and I do not wish to claim such use, broadly.

Having thus described my invention, what I claim, and desire to secure by Letters Patent of the United States, is—

1. The process of obtaining nickel and cobalt in a homogeneous and malleable form, which consists in impregnating the reduced oxides of the metals with a manganate or permanganate salt, and then smelting the impregnated oxide, 45 as described, for the purpose specified.

2. The process of obtaining nickel and cobalt in a homogeneous and malleable form, which consists in impregnating the reduced oxides of the metals with a manganate or permanganate 50 salt smelting the same, and covering the molten metal with black flux at the termination of the smelting process, substantially as described, and for the purpose specified.

3. The process of obtaining nickel and cobalt 55 in a homogeneous and malleable form, which consists in first impregnating the reduced oxides of the metals with a manganate or permanganate salt, smelting the impregnated oxide, covering the molten metal with charcoal, 60 and adding at or after the termination of the smelting process aluminium, or calcium, or calcium-zinc, or mixtures of these, substantially as and for the purpose specified.

In testimony whereof I affix my signature in 65 presence of two witnesses.

ARTUR KRUPP.

Witnesses:

JAMES RILEY WEAVER,  
CLARENCE M. HYDE.